

June 27, 1933.

B. HAYTOCK, JR

1,915,929

HOSIERY

Filed Aug. 29, 1930

FIG. II.



FIG. III.



WITNESSES  
Thomas W. Kerr, Jr.  
John A. Weidler

INVENTOR:  
Benjamin Haytock, Jr.  
BY: Fraley Paul  
ATTORNEYS.

## UNITED STATES PATENT OFFICE

BENJAMIN HAYTOCK, JR., OF EASTON, PENNSYLVANIA, ASSIGNOR TO CHIPMAN KNITTING MILLS, OF EASTON, PENNSYLVANIA, A CORPORATION OF PENNSYLVANIA

## HOSIERY

Application filed August 29, 1930. Serial No. 478,613.

This invention relates to hosiery, and has more especial reference to stockings made from silk, rayon and like yarns having a high gloss or lustre.

5 The object of my invention is to eliminate the sheen in hosiery made from gloss yarns, and at the same time to improve the appearance and the wearing qualities of the stockings.

10 The indicated desideratum I attain, by initially hard twisting, in one direction, the majority of the component threads of which the yarn is composed and the remainder of the component threads initially in the re-

15 verse direction, and subsequently hard twisting the component threads together to form the yarn. By such hard twisting, the yarn is rendered more compact and uniform in diameter, as well as stronger with attendant

20 suppression of the light reflective smoothness characteristic of silk or rayon yarns ordinarily employed in hosiery manufacture heretofore. The fabric of a stocking made in accordance with my invention is distinctive in that objectionable lustre and emphasis 25 of the wales is entirely absent, and in that its feel and texture is akin to that of delicate crepe woven on looms.

In the drawing, Fig. I is a diagrammatic view showing the manner in which the separate component threads of the yarn are initially twisted, and how said threads are finally twined together to form the yarn.

Fig. II illustrates a full fashioned stocking made with my improved yarn; and,

Fig. III is a conventional representation of a fragment of the fabric of the stocking within the confines of the dotted rectangle at III in Fig. II.

40 In carrying out my invention, I form the yarn Y from a multiplicity of individual strands or threads of silk, rayon, or other gloss material. In the illustrated instance the yarn Y is composed of four component

45 strands designated, respectively, by the numerals 5, 6, 7 and 8, in Fig. I. These separate strands 5, 6, 7 and 8 may, in turn, be composed of two or more fibres or filaments 5a, 6a, 7a and 8a, also as shown in Fig. I.

50 The majority of the threads—in this case the

three threads 5, 6 and 7—I initially twist individually all in the same direction, i. e., to the left between twenty and fifty turns to the inch. The fourth or remaining thread 55 8 I twist in the opposite direction or to the right between five and fifty turns per inch. To form the yarn Y, I subsequently twist the four threads 5-8 together in the same direction as the thread 8, i. e. to the right between twenty and fifty turns per inch. As a concrete example, a yarn Y having all the attributes hereinbefore pointed out, may be had by twisting the component threads 5, 6 and 7 individually thirty-six turns to the 60 inch, the thread 8 twenty-five turns to the 65 inch, and combining the threads by twisting them together thirty-two turns to the inch. Obviously, the directions of twists are immaterial provided that the described relation as between the twists of the threads 5-8 and 70 the final twist of the yarn Y is adhered to. In other words, the threads 5, 6 and 7, may be twisted to the right, and the strand 8 to the left, and the threads afterwards combined 75 by twisting them to the left to form the yarn Y.

For the purpose of diversification in my new stocking, I preferably knit the top or welt portion W and a margin W' immediately adjacent thereto, of ordinary silk or rayon yarn, and the body B of the stocking of hard twisted silk or rayon yarn Y prepared as above explained. The distinction between the contiguous portions W' and B of the stocking fabric will be readily recognized from the conventional representation of Fig. III. As shown, the fabric portion W' appears coarse with its wales sharply emphasized and with the cheeks of its loops L' flat, broad and straight due to the light twist (which is usually about two or three turns per inch in the yarn) and therefore highly reflective of light. On the other hand, in the portion B of the stocking made from the thinner yarn Y, the loops L are more open and their exposed cheeks round with the surface of the loops broken up and the gloss correspondingly minimized in consequence of the hard twist of the separate threads 95 5-8 constituting side yarn Y and the final 100

yarn twist by which said threads are combined. The portion B of the fabric thus takes on a delicate, subdued and crepe-like appearance, and is characterized by an entirely different feel from that of the portion W.

Having thus described my invention, I claim:

1. As a new article of manufacture, a stocking made from gloss yarn consisting of a multiplicity of separate threads whereof the majority are initially twisted individually in one direction, and the others initially twisted individually in the opposite direction, and all said threads subsequently twisted together to form the yarn.

2. As a new article of manufacture, a stocking made from gloss yarn consisting of a multiplicity of separate threads whereof the majority are initially twisted individually in one direction and the minority initially twisted individually in the opposite direction, and all the threads subsequently twisted together in the same direction as the individual threads of the minority to form the yarn.

3. As a new article of manufacture, a stocking made from gloss yarn consisting of a multiplicity of separate threads whereof the majority are initially twisted individually to the left, and the minority initially twisted individually to the right, and all said threads subsequently twisted together to form the yarn.

4. As a new article of manufacture, a stocking made from gloss yarn consisting of four separate threads whereof three are initially twisted individually in one direction and the fourth thread twisted in the opposite direction, and the four threads subsequently twisted together, to form the yarn.

5. As a new article of manufacture, a stocking made from gloss yarn consisting of four separate threads whereof three are initially twisted individually in one direction, and the fourth thread twisted in the opposite direction, and all said threads subsequently

twisted together in the same direction as the fourth thread aforesaid to form the yarn.

6. As a new article of manufacture, a stocking made from gloss yarn consisting of a multiplicity of four separate threads whereof three are initially twisted individually to the left between twenty and fifty turns per inch, and the fourth thread initially twisted between five and fifty turns per inch to the right, and all said threads subsequently twisted together between twenty-five and fifty turns per inch, to the right to form the yarn.

7. A knitted fabric made of yarn composed of a number of twisted-together strands, the majority of which have been individually given a comparatively high twist in one direction, the others individually given a comparatively low twist in the opposite direction, and the twisting together of which has been at a higher twist but in the same direction as that of the minority of strands.

8. A knitting yarn composed of a number of twisted-together strands the majority of which have been individually given a high twist in one direction and the others individually given a comparatively low twist in the opposite direction, and the twisting together of which has been at a higher twist but in the same direction as that of the minority of strands.

9. A knitting yarn composed of four strands three of which have been tightly twisted individually in one direction, the fourth strand lightly twisted in the opposite direction, and all of which are unitingly twisted together in the same direction as the fourth strand to a less number of turns per inch than the individual twists of said three strands.

In testimony whereof, I have hereunto signed my name at Easton, Pennsylvania, this 25th day of August, 1930.

BENJAMIN HAYTOCK, JR.